

## UNITED STATES PATENT OFFICE

2,676,128

PROCESS OF PREPARING NONWOVEN  
FABRIC AND PRODUCT

John Augustus Piccard, Swarthmore, Pa., assignor  
to E. I. du Pont de Nemours & Company, Wil-  
mington, Del., a corporation of Delaware

No Drawing. Application June 18, 1951,  
Serial No. 232,245

17 Claims. (Cl. 154—101)

1

This invention relates to the production of non-woven fabrics, particularly to such fabrics which are adapted for use where high strength and absence of a weave pattern are desired.

Filaments have been made from a large variety of materials, such as, e. g. cellulose acetate, viscose, copolymers of vinyl chloride and vinyl acetate, polyvinylidene chloride, copolymers of vinylidene chloride and acrylonitrile, nylon, glass, acrylic polymers and many others. These synthetic polymers have been mixed with each other and various natural fibers, such as cotton, wool and silk to produce both woven and non-woven fabrics for a great many uses.

When woven fabrics are used for certain applications such as a base or substrate for flexible coatings in the manufacture of upholstery, pocketbooks, and artificial leather in general the fabric weave pattern shows through the surface coatings and is generally undesirable. Many attempts have been made to overcome this undesirable characteristic of coated woven fabrics. The use of felts or non-woven fabrics made from various fibers and fiber combinations has been tried many times as a substrate for flexible coatings in the manufacture of various artificial leather products. The non-woven fabrics produced heretofore for this purpose have lacked sufficient tensile and tear strength or are too stiff and boardy to be of any appreciable value. Also the felts or non-woven fabrics available heretofore for this purpose have resulted in a very uneven coated surface such as an exaggerated orange peel effect.

An object of this invention is the production of non-woven fabrics which have greatly improved physical properties. A further object is the production of a non-woven fabric having improved tensile and tear strength. These and other important objects will be readily apparent as the description of the invention proceeds.

These and other important objects are accomplished according to the present invention by the provision of a non-woven fabric comprising non-fusible or relatively non-fusible fibers, which form the fabric structure, bonded together by means of certain fusible elastic polyesters defined more fully hereinafter. The relatively non-fusible fibers may consist of cotton, nylon, viscose rayon, cellulose acetate, polyethylene terephthalate, polymers of acrylonitrile, copolymers containing at least 85% acrylonitrile, wool, glass and mixtures thereof.

The term "non-fusible" or "relatively non-fusible" as used throughout the specification and appended claims refers to a structural fiber having a fusion temperature higher than the fusible polyester, referred to hereinafter as the binder. The differential in the temperature at which the structural fiber and the binder develop adhesive

properties should preferably be about 50° F. for commercial operations. Under certain controlled conditions this temperature differential may be less than about 50° F.

5 The copolymers employed for the fusible or binding material are similar to those prepared by copolymerizing under melt polymerization conditions and within certain composition limits hereinafter set forth, at least one acyclic dicarboxylic acid of the formula



wherein X is a linear chain composed of 4 to 9 atoms, in the chain of which not more than 15 three may be oxygen atoms and the remaining are hydrocarbon carbon atoms, any two such oxygen atoms being separated by at least two such carbon atoms, the hydrocarbon carbon atoms being saturated and containing a total of not more than three hydrocarbon carbon atoms 20 as side chain substituents, with at least one symmetrical aromatic dibasic acid from the group consisting of terephthalic acid, bibenzoic acid, ethylene bis p-oxybenzoic acid, tetramethylene bis p-oxybenzoic acid, and 2,6-naphthalic acid 25 and with a polymethylene glycol of the formula



wherein n is a whole number from 2 to 6 inclusive. Fibers prepared from these copolymers by the conventional melt or solvent spinning technique exhibit an elastic recovery, after orientation by cold drawing, of the order of 90% or better within one minute after an extension of 30 100%. The copolymers per se are the invention of Mark D. Snyder and are disclosed and claimed in copending application Serial No. 150,811 filed March 20, 1950, now U. S. Patent 2,623,033.

35 40 The relative amounts of aliphatic and aromatic acids to be used are critical in preparing copolymers for the purpose of this invention, since if too much of either one is used the copolyester tends to be too crystalline to produce highly elastic polymers. Therefore, to make the elastic copolyester for the purpose of this invention, it is necessary that the aromatic acid comprise at least 30% and not more than 70% by weight of the total acid component of final polymer.

45 50 A preferred range is 55-65% of the aromatic acid. It is a simple matter to obtain any desired ratio of acid components in any one copolyester. The acids will be present in the final polymer in the same ratio as they were present in the initial reactants provided an excess of glycol is used. It should be understood, of course, that many combinations of these aliphatic and aromatic acids 55 may be used. Thus, two or more aliphatic and/or two or more aromatic acids may be used to form the copolyester. It is also to be understood that

2

the ester-forming derivatives of these acids can be used in place of, and are the full equivalents of the acids described above as is generally the case in the manufacture of linear polyesters.

In addition to the copolymers described above and disclosed in copending application Serial No. 150,811, now U. S. Patent 2,623,033, the melt mixtures of polyesters and copolymers described in copending Serial No. 150,812 filed March 20, 1950, by M. D. Snyder, now U. S. Patent 2,623,031, 5 may also be used as the binding medium for the non-fusible structural fibers. The melt-blends are prepared by first preparing the copolymer described above and thereafter melt-blending the copolymer thus formed with an aromatic polyester prepared by melt polymerizing a symmetrical aromatic dibasic acid from the group consisting of terephthalic acid, bibenzoic acid, tetramethylene bis p-oxybenzoic acid, and 2,6-naphthalic acid, and a polymethylene glycol of the 20 formula  $\text{HO}(\text{CH}_2)_n\text{OH}$ ,  $n$  being a whole number from 2 to 6 inclusive. Preferably, the same aromatic dibasic acid used in the copolymer is used in the polyester. As in the case of the copolymer, the aromatic acid component of the 25 melt-blend of the polyester and copolymer should be at least 30% and not more than 70% on a weight basis.

A preferred embodiment of this invention is carried out by preparing non-woven fabrics by 30 intermingling non-fusible structural fibers such as cotton, viscose rayon, cellulose acetate, nylon, polyethylene glycol terephthalate, polymers of acrylonitrile, copolymers containing at least 85% acrylonitrile, wool, and glass, with the polyester 35 fibers described above. The blending of the fibers is carried out mechanically or manually in accordance with well established procedures in the textile art. An alternate method is to introduce the copolymer binder in the form of a solution into a preformed mat of structural fibers which permeates the fibers and binds them together upon evaporation of the solvent. Another alternate method is to distribute the polyester 40 binder throughout the assembly of preformed bats of structural fiber in the form of finely divided particles and then activating the adhesive properties of the polyester by subjecting the assembly to heat and pressure and/or by treatment with a solvent for the polyester. Still another 45 alternate method is to introduce the binder throughout the structural fiber mat in the form of an aqueous suspension which may be fused or dissolved after drying by subjecting the impregnated mat to heat and pressure and/or a solvent 50 for the binder.

In the preferred practice a plurality of the loosely bound webs from the card or other mat forming equipment are superposed in parallel arrangement or they may be crosslapped at right 55 angles. The superposed webs are then

subjected to heat and pressure by passing between heated calender rolls under pressure or pressed between heated plates. The heat required must be sufficient to render the polyester fiber adhesive and have no appreciable effect on the relatively non-fusible or structural fibers. In actual practice a plurality of single webs from the card are superposed in parallel arrangement or alternately crosslapped in a manner well known in the art of felt making.

For the purpose of direct comparison the following specific examples were carried out using substantially the same length staples at constant denier.

#### EXAMPLE I

Monofilaments were prepared by melt spinning a copolymer consisting of 40 parts ethylene glycol sebacate per 60 parts of ethylene glycol terephthalate. The copolymer had a fusion temperature of approximately 320° F. The copolymer fiber was cut into staple of approximately 1½ inch length. After this staple was opened it was thoroughly mixed with an equal quantity of long staple cotton fibers of approximately 1½ inch length. This mixture was then carded in the form of a web weighing approximately .66 ounce per square yard in a fashion usually employed in the manufacture of non-woven fabrics. Twelve separate webs were superposed in such a manner that alternate webs were crosslapped at substantially right angles. The entire assembly was pressed for one minute between the platens of a hydraulic press at a temperature of 365° F. and at a pressure of 400 p. s. i. The felt produced was 15 to 20 mils thick and weighed approximately 8.0 ounces/square yard. It was suitable for the applications mentioned hereinafter.

The copolymer in this example may be prepared in accordance with the disclosure in copending application Serial No. 150,811 filed March 20, 1950, now U. S. Patent 2,623,033.

#### EXAMPLE II

Another felt was made in the same manner as described in Example I except the ratio of copolymer fibers to cotton fibers was 1 to 2.

#### EXAMPLE III

Another felt was produced in the same manner as described in Example I except the ratio of copolymer fibers to cotton fibers was 1 to 3.

#### EXAMPLE IV

Another felt was produced in the same manner as described in Example I except the ratio of copolymer fibers to cotton fibers was 1 to 4.

The following table is a summary of the physical properties of the felts described in Examples I to IV.

Table I

| Example  | Ratio of Structural Fiber to Binder Fiber | Pressing Temperature, ° F. | Tensile <sup>1</sup> (1" Strip) (lbs.) |          | Tear <sup>1</sup> (lbs.) |          | Percent Elongation <sup>1</sup> to Breaking Point (1" Strip), W/F | Hand                                    |
|----------|-------------------------------------------|----------------------------|----------------------------------------|----------|--------------------------|----------|-------------------------------------------------------------------|-----------------------------------------|
|          |                                           |                            | W/F <sup>2</sup>                       | W plus F | W/F                      | W plus F |                                                                   |                                         |
| I.....   | 1 to 1.....                               | 365                        | 50/63                                  | 113      | 3.3/3.5                  | 6.8      | 12/7                                                              | Boardy.                                 |
| II.....  | 2 to 1.....                               | 365                        | 25/43                                  | 68       | 3.7/4.7                  | 8.4      | 10/13                                                             | Sl. Board.                              |
| III..... | 3 to 1.....                               | 365                        | 33/22                                  | 65       | 3.5/3.2                  | 6.7      | 8.5/8.5                                                           | Soft.                                   |
| IV.....  | 4 to 1.....                               | 365                        | 8/18                                   | 26       | 3.0/2.7                  | 5.7      | 4/10                                                              | Loosely bound and low tensile strength. |

<sup>1</sup> The tensile strength, tongue tear and elongation tests were carried out in accordance with the procedures described in ASTM, D39-49.

<sup>2</sup> The letters "W" and "F" refer to the conventional warp and filler direction of woven fabrics. In this instance and hereinafter the "W" refers to the machine direction of the non-woven fabric and the "F" refers to the cross-machine direction.

## EXAMPLE V

A non-woven fabric was prepared in the same manner as described in Example I in which the structural fiber (non-binding) was 3.0 denier nylon monofilament staple approximately 1½ inches long. Three parts by weight of this staple were mixed with one part of the copolyester staple fiber referred to in Example I. The mixed staples were carded and formed into a web. Twelve separate webs were crosslapped, and compacted by passing between calender rolls heated to 265° F. at a rate of 6 ft. per minute, with the calender roll's opened to 4 mils. The resulting felt was approximately 8.0 oz./sq. yd. and 16 mils thick. It was smooth and exhibited unusually high tensile and tear strength as shown in Table II.

The nylon polymer in the above example is a synthetic linear polyamide resulting from the reaction of hexamethylene diamine and adipic acid and may be produced in accordance with the teachings in U. S. Patents 2,071,250 and 2,071,251.

## EXAMPLE VI

A non-woven fabric was produced in the same manner as described in Example V except the relatively non-fusible structural fiber was a polyester of ethylene glycol and terephthalic acid and the binding fiber was the copolyester referred to in Example I and nine separate webs were employed in crosslapped relation. Three parts of the polyester fiber were blended with one part of copolyester fiber. The compacting was carried out by calendering in the same manner as described in Example V. The non-woven fabric weighed approximately 8.0 ounces/square yard and was soft and flexible.

The polyethylene terephthalate may be produced in accordance with the disclosure in U. S. Patent 2,465,319.

## EXAMPLE VII

A non-woven fabric was prepared in the same manner as described in Example V except viscose rayon 3.0 denier, 1½ inch staple monofilaments were used as the structural fiber.

## EXAMPLE VIII

Example V was repeated using 1½ inch long staple cotton fiber in place of the nylon as the structural fiber.

The following Table II summarizes the physical properties of the non-woven fabrics referred to in Examples V to VIII.

Table II

| Example | Structural Fiber                                    | Binding Fiber                      | Properties of Non-Woven Fabric |          |                    |          |                                                      |                    |
|---------|-----------------------------------------------------|------------------------------------|--------------------------------|----------|--------------------|----------|------------------------------------------------------|--------------------|
|         |                                                     |                                    | Tensile (lbs. per 1" Strip)    |          | Tongue Tear (lbs.) |          | Percent Elongation to Breaking Point (1" Strip), W/F | Hand               |
|         |                                                     |                                    | W/F                            | W plus F | W/F                | W plus F |                                                      |                    |
| V       | Nylon                                               | Copolyester, Same as in Example I. | 67/88                          | 155      | 27/31              | 58       | 75/80                                                | Soft and Flexible. |
| VI      | Polyester of Ethylene Glycol and Terephthalic Acid. | do.                                | 20/52                          | 72       | 8.5/10.5           | 19       | 63/63                                                | Do.                |
| VII     | Viscose Rayon                                       | do.                                | 18/34                          | 52       | 1/5                | 6        | 20/16                                                | Do.                |
| VIII    | Cotton                                              | do.                                | 14/17                          | 31       | 3.7/4              | 7.7      | 22/22                                                | Do.                |

## EXAMPLE IX

A non-woven felt-like fabric was produced by carding the nylon fiber referred to in Example V into the form of a web weighing approximately 75

ounces per square yard. Eight separate webs were superposed and then placed between two sheets of 80 mesh wire screen. The assembly was subjected to moderate pressure by hand to compact the superposed plies. The entire assembly was then dipped into a 5% solution of a copolymer of 60 parts of ethylene glycol terephthalate and 40 parts of ethylene glycol sebacate dissolved in chloroform. The assembly was then removed from the solution and the excess solution was allowed to drain off. To facilitate saturation of the superposed webs the assembly was subjected to the action of a hand roller on each side. The assembly was then dried at 250° F. until the chloroform was evaporated. The wire screens were then removed from the web and the dried web further condensed by passing between pressure rolls heated to about 265° F. A soft, high strength unitary non-woven felt was obtained.

## EXAMPLE X

A non-woven felt-like fabric is produced by forming a web of long staple (1½ inch cotton fibers) and superposing eight separate webs to form a bat. Finely divided copolyester of 60 parts ethylene glycol terephthalic acid and 40 parts ethylene glycol sebacate is distributed throughout the assembly. The entire assembly consists of about 75% cotton fibers and 25% copolyester on a weight basis. The finely divided copolyester is distributed on the surface and at least to some extent throughout each individual web. The entire assembly is next pressed between heated platens at a temperature of about 350° F. for a period of 1 minute. The resultant product is a soft high strength non-woven fabric suitable for use as substrate for flexible coatings and other uses where high strength non-woven fabrics are required.

## EXAMPLE XI

A non-woven felt-like fabric was produced by blending the following fibers:

|    |                                                                                                          | Parts by weight |
|----|----------------------------------------------------------------------------------------------------------|-----------------|
| 45 | Nylon (1½" staple, 3.0 denier)                                                                           | 1               |
|    | Polyester of ethylene glycol and terephthalic acid (1½" staple, 3.0 denier)                              | 1               |
|    | Copolyester of 60 ethylene glycol terephthalate and 40 ethylene glycol sebacate (1½" staple, 3.0 denier) | 1               |
| 50 |                                                                                                          |                 |

The blended fibers were carded in the form of a web weighing about ¾ ounce per square yard. Twelve separate webs were superposed, the first four webs in parallel arrangement, the second four in parallel arrangement and at right

angles to the first four and the third four were in parallel arrangement and at right angles to the second four. The composite assembly was compacted by passing between even speed high

pressure rolls heated to about 265° F. and set about 4 mils apart.

The assembly was compacted to approximately 15 mils thick and weighed approximately 8.0 ounces per square yard. The felt-like material had the following physical properties:

|                                       | W/F        |
|---------------------------------------|------------|
| Tongue tear                           | lbs. 31/31 |
| Tensile—1" strip                      | lbs. 74/50 |
| Per cent elongation to breaking point | 75/57 10   |

#### EXAMPLE XII

A non-woven felt-like fabric was made in the same manner as described in Example XI except the following blend of fibers was employed:

|                                                                                                          | Parts by weight |
|----------------------------------------------------------------------------------------------------------|-----------------|
| Polyacrylonitrile (1½" staple, 3.0 denier)                                                               | 3               |
| Copolyester of 60 ethylene glycol terephthalate and 40 ethylene glycol sebacate (1½" staple, 3.0 denier) | 1 20            |

Twelve carded webs were superposed with alternate sets of four webs crosslapped and the assembly compacted by passing between heated (265° F.) pressure rolls set 4 mils apart. The resulting product weighing 8.1 ounces per square yard was suitable as a substrate for flexible coatings. It had the following physical properties:

|                                           | W/F           |
|-------------------------------------------|---------------|
| Tensile strength—1" strip                 | lbs. 33/45 30 |
| Tongue tear                               | lbs. 8/13     |
| Per cent elongation to the breaking point | 45/50         |

#### EXAMPLE XIII

A non-woven felt-like fabric was produced by carding the following blend of fibers on a hand card:

|                                                                                                                                                                              | G.     |
|------------------------------------------------------------------------------------------------------------------------------------------------------------------------------|--------|
| Cellulose acetate—3.0 denier, 1½" staple                                                                                                                                     | 10.0   |
| Copolyester (same as Example I)—3.0 denier, 1½" staple                                                                                                                       | 3.0 40 |
| Melt-blend of polyethylene glycol terephthalate and a copolymer of 40 parts of ethylene glycol terephthalate and 60 parts of ethylene glycol sebacate—3.0 denier, 1½" staple | 5.0 45 |

The polyethylene glycol terephthalate and the copolymer were blended in a ratio so that the aromatic acid component was 70% by weight of the total acid component of the blend. Two separate bats about 10" square were produced from a blend of the above fibers. The two separate bats were superposed and trimmed to about 8" square. The superposed bats were pressed at about 320° F. and approximately 500 p. s. i. The assembly was firmly bonded and was a flexible felt-like fabric.

The melt-blended fibers, in the above formula, develop adhesiveness at about 350–390° F. In the above example they serve as structural fibers. When higher melting structural fibers are employed, such as, e. g. nylon, this melt-blend may be used as binding fibers.

For the purpose of this invention it is important that the structural fibers not develop any adhesiveness at the temperature at which the binder is rendered adhesive. The copolymers described above have a fusion temperature of 300–400° F. They do not have a true melting point in the ordinary sense of the word. The temperature at which adhesiveness develops depends more or less on the degree of crystallinity of the polymer and is lower than the fusion temperature. The preferred polyester binder containing 60 parts of ethylene glycol terephtha-

late and 40 parts ethylene glycol sebacate has a fusion temperature, approximately 320° F. although adhesiveness develops at a lower temperature. The invention is not to be limited to the particular temperature range mentioned above for the fusion temperature of the copolyester binder. The important thing is that the binder develop adhesiveness at about 50° F. lower than the structural fiber. The fusion temperature is not to be confused with the temperature at which adhesiveness develops. When a thermoplastic fiber is used as the structural fiber it must not lose its identity as a fiber during the processing. Nylon is particularly preferred as the structural fiber in view of its relatively high melting point (approximately 482° F.) and high tensile and tear strength. The wide difference in temperature at which adhesiveness is developed in the nylon polymer and the copolymers provides a safe operating range for the practice of this invention.

It is also possible to improve the adhesiveness of the binding fiber by treating the matted felt after the compacting operation with a volatile liquid which renders the binding fiber cementitious.

The copolymers and melt-blend of polyesters and copolymers described above are particularly useful for the purpose of this invention in view of their elastic recovery when elongated. Conventional non-woven fabrics and papers tear relatively easily when a strip is cut on one edge and the cut edges are subjected to opposing forces since the fibers are broken one at a time as the entire stress is applied to a relatively few fibers. When the non-woven fabrics employing the elastic copolymers and melt-blended polyesters and copolymers as the binding medium are cut on one edge and the cut edges are subjected to opposing forces the elastic fibers stretch and the stress is distributed over a greater number of fibers than in the case of conventional non-woven fabrics.

A commercial grade of felt weighing about 8 ounces/square yard comprising a blend of viscose rayon, cotton, and a binding fiber consisting of copolymer of 85 parts of vinyl chloride and 15 parts of vinyl acetate was subjected to the same tests as shown in Tables I and II with the following results:

|                                    | Commercial Felt, 8 oz./sq. yd. |
|------------------------------------|--------------------------------|
| 55 Tensile Strength 1" Strip (WXF) | 9×13 lbs.                      |
| Tear Strength (Tongue)             | 3.2×5.2 lbs.                   |

A comparison of the above data with Tables I and II illustrates the advantages of the products of this invention over prior art material of equal weight.

The copolymers and melt-blended copolymers and polyesters described in copending application Serial No. 150,811 and Serial No. 150,812 both filed March 20, 1950, U. S. Patents 2,623,033 and 2,623,031, respectively, when used in this invention in the form of fibers may be cold drawn, that is, permanently elongated by tensile stress in order to orient them since the oriented filaments have greater strength and elasticity. The unoriented or but slightly oriented filaments obtained by spinning under little or no stress are, however, also useful in the practice of this invention.

The various copolymers described above used

to form the non-woven fabric may be plasticized or unplasticized. If a softer binding fiber or one which develops adhesiveness at a lower temperature is desired it may be plasticized with an aryl sulfonamide, such as toluene sulfonamide or amylibenzene sulfonamide.

The proportion of thermoadhesive binder to the non-thermoadhesive fiber used in the examples illustrate the preferred proportions. Where very soft fluffy felts are desired the binder may represent as little as 10% of the total and when very stiff and boardy felts are desired the binder may represent as high as 65% of the total.

The time, temperature and pressure used in the specific examples may vary depending upon the nature of the thermoadhesive or binding fiber, particularly its softening point, and on the nature of the structural or non-thermoadhesive fibers present. For example, if a high melting filament is used as the binding fiber a relatively higher temperature and pressure will be required than if a low melting filament is used. Likewise, if a soft fabric is desired a lower pressure and/or temperature will be used than if a hard fabric is desired. Also, at higher pressures lower temperatures may be employed.

The fabrics produced in accordance with this invention can be dyed by the usual methods either by application of the dye to the formed felt or to the fibers before carding.

The physical properties of the fabric such as, e. g., its feel and tackiness may be altered, if desired, by subjecting the fabric to fluffing and steaming treatments.

The denier of the filaments which may be used in carrying out this invention may vary depending on the type and appearance of the non-woven fabric desired. While the three denier filament is preferred, filaments having a denier of one or less may be used. Fibers having a denier of 50 to 70 produce useful non-woven fabrics and where extremely coarse felt is desired, even coarser filaments having a denier of 100 to 150 may be used. The thermoadhesive binding filament and the non-thermoadhesive structural fiber may be straight or crimped.

The non-woven fabrics of this invention, depending upon the particular fibers used and upon the conditions of treatment, possess a wide range of properties which adapt the product for the different purposes for which non-woven fabrics and felts are now used. As examples of some of these uses may be mentioned the use of soft felt in wadding, slightly harder felt in coat and shoe linings, upholstery, millinery, filtering media and insulation.

The products of this invention are particularly useful as substrates for flexible coatings such as plasticized cellulose derivatives, including ethyl cellulose, cellulose nitrate, cellulose acetate, cellulose acetobutyrate, and cellulose aceto-propionate. The non-woven fabrics herein described are also useful as a base for flexible synthetic resin coatings comprising polyvinyl acetals, polyvinyl halides, polymethacrylic acid esters, amino aldehyde resins and alkyd resins. The present invention is particularly adapted to the production of high strength substrates for plasticized polyvinyl chloride coatings used as upholstery fabrics. The flexible coatings may be applied from solutions or deposited from suspensions in which the film former of the coating is suspended in a non-solvent for said film former, and the film formed by heating after it is applied to the substrate. Where the film former is sus-

pended in a plasticizer, such compositions are referred to as "plastisols." Where the suspending medium is an organic volatile liquid such compositions are referred to as "organosols." 5 Also the flexible coatings may be applied by the well known calendering methods. The flexible coatings may be applied to either or both sides of the non-woven fabric. The absence of a weave pattern in the non-woven fabric makes it particularly useful as a substrate for flexible coatings where a fabric weave pattern is objectionable.

The coated products referred to above are disclosed and claimed in a copending application

15 S. N. 232,247, filed June 18, 1951, by E. A. Rodman, It is apparent that many widely different embodiments of this invention may be made without departing from the spirit and scope thereof and, therefore, it is not intended to be limited 20 except as indicated in the appended claims.

I claim:

1. A non-woven fabric comprising compacted structural staple fibers selected from the group consisting of cotton, nylon, viscose rayon, cellulose acetate, polyethylene terephthalate, polymers of acrylonitrile, wool and glass, bound together by a binding material comprising a linear copolyester of (a) at least one polymethylene glycol ester of an acyclic dicarboxylic acid of the 30 formula



wherein X is a linear chain composed of 4 to 9 atoms, in the chain of which not more than 3 may be oxygen atoms and the remaining are hydrocarbon carbon atoms, any two such oxygen atoms being separated by at least two such carbon atoms, the hydrocarbon carbon atoms being saturated and containing a total of not more than three hydrocarbon carbon atoms as side chain 35 substituents, with (b) at least one polymethylene glycol ester of a symmetrical aromatic dibasic acid from the group consisting of terephthalic acid, bibenzoic acid, ethylene bis-p-oxy-benzoic acid, tetramethylene bis-p-oxy-benzoic acid and 40 2,6-naphthalic acid, the aromatic acid comprising from 30% to 70% by weight of the acid components of the copolyester and the polymethylene glycol component of (a) and (b) having from 2 to 6 carbon atoms, the binding material being 45 present in amount between 10% and 65%, based 50 on the combined weight of the binding material and the structural fibers.

2. The product of claim 1 in which the aromatic acid component of the copolyester represents 55-65% of the acid components of the copolyester.

3. The product of claim 1 in which the binder is a copolyester of 40 parts of ethylene glycol sebacate and 60 parts of ethylene glycol terephthalate.

4. The product of claim 1 in which the structural fiber is nylon and the binder is a copolyester of 40 parts of ethylene glycol sebacate and 60 parts of ethylene glycol terephthalate.

5. The process of preparing non-woven fabrics which comprises matting staple fibers selected from the group consisting of cotton, nylon, viscose rayon, cellulose acetate, polyethylene terephthalate, polymers of acrylonitrile, wool and glass, mixing a dry binder with said matted staple fibers, said binder comprising a linear copolyester of (a) at least one polymethylene glycol ester of an acyclic dicarboxylic acid of the 70 formula



wherein X is a linear chain composed of 4 to 9 atoms, in the chain of which not more than 3 may be oxygen atoms and the remaining are hydrocarbon carbon atoms, any two such oxygen atoms being separated by at least two such carbon atoms, the hydrocarbon carbon atoms being saturated and containing a total of not more than three hydrocarbon carbon atoms as side chain substituents, with (b) at least one polymethylene glycol ester of a symmetrical aromatic dibasic acid from the group consisting of terephthalic acid, bibenzoic acid, ethylene bis p-oxy-benzoic acid, tetramethylene bis p-oxy-benzoic acid and 2,6-naphthalic acid, the aromatic acid comprising from 30% to 70% by weight of the acid components of the copolyester and the polymethylene glycol component of (a) and (b) having from 2 to 6 carbon atoms, and subjecting the mat and binder to heat and pressure sufficient to activate the adhesiveness of the copolyester, the binding material being present in amount between 10% and 65%, based on the combined weight of the binding material and the structural fibers.

6. The process of claim 5 in which the aromatic acid component of the copolyester represents 55-65% of the acid component of the copolyester.

7. The process of claim 5 in which the binder is a copolyester of 40 parts of ethylene glycol sebacate and 60 parts of ethylene glycol terephthalate.

8. The process of claim 5 in which the structural fiber is nylon and the binder is a copolyester of 40 parts of ethylene glycol sebacate and 60 parts of ethylene glycol terephthalate.

9. The process of preparing non-woven fabrics which comprises matting a mixture of structural fibers and dry binding fibers, said structural fibers selected from the group consisting of cotton, nylon, viscose rayon, cellulose acetate, polyethylene terephthalate, polymers of acrylonitrile, wool and glass, said binder fibers comprising a linear copolyester of (a) at least one polymethylene glycol ester of an acyclic dicarboxylic acid of the formula



wherein X is a linear chain composed of 4 to 9 atoms, in the chain of which not more than 3 may be oxygen atoms and the remaining are hydrocarbon carbon atoms, any two such oxygen atoms being separated by at least two such carbon atoms, the hydrocarbon carbon atoms being saturated and containing a total of not more than three hydrocarbon carbon atoms as side chain substituents, with (b) at least one polymethylene glycol ester of a symmetrical aromatic dibasic acid from the group consisting of terephthalic acid, bibenzoic acid, ethylene bis p-oxy-benzoic acid, tetramethylene bis p-oxy-benzoic acid and 2,6-naphthalic acid, the aromatic acid comprising from 30% to 70% by weight of the acid components of the copolyester and the polymethylene glycol component of (a) and (b) having from 2 to 6 carbon atoms, and subjecting the matted mixture to heat and pressure sufficient to activate the adhesiveness of the copolyester, the binding fibers being present in amount between 10% and 65% based on the combined weight of the binding fibers and the structural fibers.

10. The process of claim 9 in which the aromatic acid component of the copolyester represents 55-65% of the acid component of the copolyester.

11. The process of claim 9 in which the binder fiber is a copolyester of 40 parts of ethylene glycol

sebacate and 60 parts of ethylene glycol terephthalate.

12. The process of claim 9 in which the structural fiber is nylon and the binder fiber is a copolyester of 40 parts of ethylene glycol sebacate and 60 parts of ethylene glycol terephthalate.

13. A non-woven fabric comprising compacted structural staple fibers selected from the group consisting of cotton, nylon, viscose rayon, cellulose acetate, polyethylene terephthalate, polymers of acrylonitrile, wool and glass bound together by a melt blend of (1) a linear copolyester of (a) at least one polymethylene glycol ester of an acyclic dicarboxylic acid of the formula



wherein X is a linear chain composed of 4 to 9 atoms, in the chain of which not more than 3 may be oxygen atoms and the remaining are hydrocarbon carbon atoms, the hydrocarbon carbon atoms being saturated and containing a total of not more than three hydrocarbon carbon atoms as side chain substituents, with (b) at least one polymethylene glycol ester of a symmetrical aromatic dibasic acid from the group consisting of terephthalic acid, bibenzoic acid, ethylene bis p-oxy-benzoic acid, tetramethylene bis p-oxy-benzoic acid and 2,6-naphthalic acid, the aromatic acid comprising from 30% to 70% by weight of the acid components of the copolyester and (2) a linear polyester of at least one linear polymethylene glycol ester of a symmetrical aromatic dibasic acid from the group consisting of terephthalic acid, bibenzoic acid, tetramethylene bis p-oxy-benzoic acid, and 2,6-naphthalic acid, the polymethylene glycol component of (1) and (2) having 2 to 6 carbon atoms, the total aromatic acid content of the blend being from 30% to 70% by weight of the acid components of the blend, the binding material being present in amount between 10% and 65%, based on the combined weight of the binding material and the structural fibers.

14. A non-woven fabric comprising staple nylon fibers bound together by a linear copolyester of ethylene glycol sebacate and ethylene glycol terephthalate.

15. The product of claim 14 in which the binder comprises 40 parts of the ethylene glycol sebacate and 60 parts of the ethylene glycol terephthalate.

16. The process of preparing non-woven fabrics which comprises matting staple nylon fibers, mixing therewith a dry linear copolyester of ethylene glycol sebacate and ethylene glycol terephthalate, and subjecting the assembly to heat and pressure sufficient to render the copolyester adhesive.

17. The process of claim 16 in which the copolyester is introduced as dry particles.

60 References Cited in the file of this patent

UNITED STATES PATENTS

| Number    | Name      | Date           |
|-----------|-----------|----------------|
| 2,277,049 | Reed      | Mar. 24, 1942  |
| 2,357,392 | Francis   | Sept. 5, 1944  |
| 2,476,282 | Castellan | July 19, 1949  |
| 2,543,101 | Francis   | Feb. 27, 1951  |
| 2,544,019 | Heritage  | Mar. 6, 1951   |
| 2,569,169 | Heritage  | Sept. 25, 1951 |

70 FOREIGN PATENTS

| Number  | Country       | Date         |
|---------|---------------|--------------|
| 623,309 | Great Britain | May 16, 1949 |